

Aug. 17, 1948.

P. L. SPENCER

2,447,038

CATHODE STRUCTURE

Filed Oct. 31, 1945



INVENTOR  
PERCY L. SPENCER  
BY Elmer J. Gorn  
ATTY.

## UNITED STATES PATENT OFFICE

2,447,038

## CATHODE STRUCTURE

Percy L. Spencer, West Newton, Mass., assignor to  
 Raytheon Manufacturing Company, Newton,  
 Mass., a corporation of Delaware

Application October 31, 1945, Serial No. 625,731

5 Claims. (Cl. 250—27.5)

1

This invention relates to cathode structures for electron-discharge devices, and while not limited thereto, it is especially suitable for use in electron-discharge devices of the magnetron type.

One of the disadvantages of existing cathode structures, which ordinarily consist of metallic cores provided with highly electron-emissive coatings, is the development, in the coatings, of hot spots. These hot spots are caused by the uneven thermal conductivity between the core and the coating, and result in rapid deterioration of the structure as an electron emitter.

It is, therefore, one of the objects of the present invention to provide a cathode structure having substantially uniform thermal conductivity throughout.

It is a further object of the present invention to provide a cathode structure in which there is improved coherence between the core and the coating thereof.

These, and other objects of the present invention, which will become more apparent as the detailed description thereof progresses, are attained, briefly, in the following manner:

In accordance with the present invention, a metallic base member is covered with a metallic gauze. A metallic cementing agent, dispersed in a suitable binder, is applied to the composite base member and gauze, which are then heated to a temperature sufficient to drive off the binder and cause the cementing agent to sinter and bind the gauze to the base member. The resulting intimate contact between the gauze and the base member gives rise to substantially uniform, high thermal conductivity throughout. In addition, the gauze surface being porous, a subsequently applied electron-emissive coating fills the interstices thereof, thereby assuring greater coherence between the coating and the cathode core.

In the accompanying specification there shall be described, and in the annexed drawing shown, an illustrative embodiment of the electron-discharge device of the present invention. It is, however, to be clearly understood that the present invention is not to be limited to the details herein shown and described for purposes of illustration only, inasmuch as changes therein may be made without the exercise of invention, and within the true spirit and scope of the claims hereto appended.

In said drawing, the single figure is a longitudinal sectional view of a cathode structure made in accordance with the principles of the present invention.

Referring now more in detail to the aforesaid

illustrative embodiment of the present invention, with particular reference to the drawing illustrating the same, the numeral 10 generally designates a cathode structure including a base member in the form of a metallic, preferably nickel, sleeve 11. Said sleeve 11 is surrounded by a metallic, preferably nickel, gauze 12 which, as herein shown in the drawing, has been greatly exaggerated.

10 In order to so bind the gauze to the sleeve as to assure good thermal conductivity therebetween throughout, a metallic cementing agent, for example, nickel powder, dispersed in a suitable binder, such as a nitro-cellulose amylacetate binder, is deposited, as by spraying, over the composite sleeve and gauze.

15 The whole is then heated, in a gaseous atmosphere adapted to prevent oxidation, for example, hydrogen, to a temperature sufficient to drive off the binder and cause the cementing agent to sinter, thereby fusing the gauze to the sleeve. The sintered cementing agent has been designated in the drawing by the reference character 13.

20 Thereafter, the structure is provided with any preferred electron-emissive coating 14, for example, a mixture of barium and strontium carbonates dispersed in a suitable carrier. This coating may be sprayed onto the structure, and 30 will flow into and fill the interstices of the gauze 12.

The structure is completed by providing the same with a suitable heating filament 15.

25 This completes the description of the aforesaid 35 illustrative embodiment of the present invention. It will be noted that the cathode structure of the present invention provides substantially uniform thermal conductivity between the electron-emissive coating and the cathode core, whereby the

40 formation of hot spots is eliminated. It will further be noted that the porous character of the surface receiving the electron-emissive coating provides improved coherence between said coating and the core.

45 Other objects and advantages of the present invention will readily occur to those skilled in the art to which the same relates.

What is claimed is:

50 1. A cathode structure comprising: a metallic core; a metallic gauze bound to said core by a fused metallic powder; and an electron-emissive coating deposited over said gauze.

2. A cathode structure comprising: a metallic core; a similarly metallic gauze bound to said core

by a fused, similarly metallic powder; and an electron-emissive coating deposited over said gauze.

3. A cathode structure comprising: a nickel core; a nickel gauze bound to said core by a fused nickel powder; and an electron-emissive coating deposited over said gauze.

4. A cathode core comprising: a metallic base member; and a metallic gauze bound to said base member by a fused metallic powder.

5. A cathode core comprising: a nickel base member; and a nickel gauze bound to said base member by a fused nickel powder.

## REFERENCES CITED

The following references are of record in the file of this patent:

## UNITED STATES PATENTS

| Number    | Name                  | Date          |
|-----------|-----------------------|---------------|
| 2,075,122 | Loewe et al. -----    | Mar. 30, 1937 |
| 2,154,298 | Ayer -----            | Apr. 11, 1939 |
| 2,251,410 | Koehring et al. ----- | Aug. 5, 1941  |
| 2,273,763 | Rerink et al. -----   | Feb. 17, 1942 |
| 2,359,361 | Gleszer et al. -----  | Oct. 3, 1944  |

## FOREIGN PATENTS

| Number     | Country         | Date         |
|------------|-----------------|--------------|
| 15 108,740 | Australia ----- | Oct. 8, 1937 |

PERCY L. SPENCER.